

Patented Mar. 11, 1947

2,417,118

# UNITED STATES PATENT OFFICE

2,417,118

## COMPOSITION OF MATTER

Rush F. McCleary and Stiles M. Roberts, Beacon, N. Y., assignors, by mesne assignments, to The Texas Company, New York, N. Y., a corporation of Delaware

No Drawing. Application August 16, 1941,  
Serial No. 407,234

10 Claims. (Cl. 260—609)

1

This invention relates to oil-soluble hydroxy aromatic or mercapto aromatic methylene thio ethers and/or the metal derivatives thereof, and to a process for preparing the same.

This invention is a continuation-in-part of the invention as described and claimed in the copending application of Rush F. McCleary and Stiles M. Roberts, S. N. 393,244, filed May 13, 1941.

The invention is based upon the discovery of a novel class of compounds which may be broadly described as oil-soluble or oil-miscible hydroxy aromatic or mercapto aromatic methylene thio ethers and/or the metal derivatives thereof which, when incorporated in a mineral lubricating oil in sufficient quantities, impart certain advantageous and desirable properties thereto, particularly with respect to inhibition of corrosion and oxidation and the prevention of undesirable deposition upon the engine parts. The resulting lubricating oil compositions containing small proportions of these compounds are described and claimed in the copending application of Rush F. McCleary and Stiles M. Roberts, S. N. 393,244, filed May 13, 1941.

The compounds of the present invention may be described as that class of aromatic compounds which contain at least one radical of the type  $-\text{CH}_2-\text{S}-\text{R}_1$  attached to a nuclear carbon atom and at least one hydroxyl (OH) or sulfhydryl (SH) radical or their metal salts. Specifically these compounds may be represented by the following structural formula



in which R may be a hydrogen, alkyl, aryl, cycloalkyl, aralkyl or naphthyl radical, and  $\text{R}_1$  may be an alkyl, aryl, cycloalkyl, aralkyl or naphthyl radical. These radicals may contain further substituents which do not affect the oil-solubility of the compound, as, for example, halogen, sulfur, oxygen, or nitrogen derivatives.  $\text{X}$  may be either an hydroxyl (OH) or sulfhydryl (SH) radical or metal salts thereof, and  $n$ ,  $y$  and  $z$  are integers of 1 or more.  $y$  and  $z$  are usually either 1, 2, 3 or 4, whereas  $n$  may be either 1, 2 or 3, depending upon the valences of the aromatic nucleus not satisfied by other substituents or residual hydrogen. The aromatic nucleus diagrammatically shown may be substituted by a naphthyl, anthracyl or any other condensed aromatic nucleus. The positions of the substituents are purely diagrammatic and may be connected

2  
to any position in the aromatic nucleus. The metal derivatives of this class of compounds which are formed by the substitution of the replaceable hydrogen in the hydroxyl radical (OH) or the sulfhydryl radical (SH) include any of the following metals: sodium, potassium, lithium, calcium, barium, strontium, magnesium, zinc, iron, cobalt, nickel, aluminum, manganese, and chromium.

As illustrating the type of compounds within the scope of the above classification, the following compounds are presented, together with their relationship to the general classification. It is to be understood that the above-mentioned metals may be substituted for the replaceable hydrogen in the following compounds and that the scope of the present invention is not limited to the following specific compounds or their metal salts:

$R=alkyl, R_1=alkyl$

$n,y,z=1, X=OH$

Amylthiomethyl tridecyl phenol

$X=SH$

Amylthiomethyl tridecyl thiophenol

$n,y=1, z=2, X=OH$

Di (butylthiomethyl) octyl phenol

$X=SH$

Di (butylthiomethyl) octyl thiophenol

$n=1, y=2, z=1, X=OH$

Amylthiomethyl dioctadecyl naphthol

$X=SH$

Amylthiomethyl dioctadecyl thionaphthol

$n=1, y,z=2, X=OH$

Di (octylthiomethyl) diethyl phenol

$X=SH$

Di (octylthiomethyl) diethyl thiophenol

$n=3, y,z=1, X=OH$

Amylthiomethyl undecyl pyrogallol

$n=2, y=1, z=2, X=OH$

Di (amylthiomethyl) undecyl resorcinol

$n=3, y=2, z=1, X=OH$

Amylthiomethyl diethyl pyrogallol

In the following compounds  $\text{X}$  is an hydroxyl radical, although the corresponding thio compounds, e. g., where  $\text{X}$  is a sulfhydryl radical, may also be used:

$R=hydrogen, R_1=alkyl$

## 3

|                                            |    |
|--------------------------------------------|----|
| $n=1, y=3, z=2$                            |    |
| Di (butylthiomethyl) phenol                |    |
| $n=1, y=2, z=3$                            |    |
| Tri (octylthiomethyl) phenol               | 5  |
| $n,y,z=2$                                  |    |
| Di (amylthiomethyl) resorcinol             |    |
| $n=2, y=1, z=3$                            | 10 |
| Tri (amylthiomethyl) resorcinol            |    |
| $R=cycloalkyl, R_1=alkyl$                  |    |
| $n,y,z=1$                                  |    |
| Butylthiomethyl cyclohexyl phenol          | 15 |
| $n,y=1, z=2$                               |    |
| Di (butylthiomethyl) cyclohexyl phenol     |    |
| $n=1, y=2, z=1$                            | 20 |
| Butylthiomethyl di-cyclohexyl phenol       |    |
| $n=2, y,z=1$                               |    |
| Octylthiomethyl cyclohexyl resorcinol      |    |
| $n=2, y=1, z=2$                            | 25 |
| Di (octylthiomethyl) cyclohexyl resorcinol |    |
| $n,y=2, z=1$                               |    |
| Octylthiomethyl di-cyclohexyl resorcinol   |    |
| $R=aralkyl, R_1=alkyl$                     |    |
| $n,y,z=1$                                  |    |
| Hexylthiomethyl benzyl naphthol            |    |
| $n,y=1, z=2$                               |    |
| Di (hexylthiomethyl) benzyl naphthol       |    |
| $n=1, y=2, z=1$                            |    |
| Hexylthiomethyl dibenzyl naphthol          |    |
| $n=2, y,z=1$                               |    |
| Hexylthiomethyl benzyl resorcinol          |    |
| $n=2, y=1, z=2$                            | 40 |
| Di (hexylthiomethyl) benzyl resorcinol     |    |
| $n,y=2, z=1$                               |    |
| Hexylthiomethyl dibenzyl resorcinol        |    |
| $R=aryl, R_1=alkyl$                        |    |
| $n,y,z=1$                                  |    |
| Amylthiomethyl phenyl phenol               |    |
| $n,y=1, z=2$                               | 50 |
| Di (amylthiomethyl) phenyl phenol          |    |
| $n=1, y=2, z=1$                            |    |
| Amylthiomethyl diphenyl phenol             |    |
| $n=2, y,z=1$                               | 55 |
| Amylthiomethyl phenyl resorcinol           |    |
| $n=2, y=1, z=2$                            |    |
| Di (amylthiomethyl) phenyl resorcinol      |    |
| $n,y=2, z=1$                               |    |
| Amylthiomethyl diphenyl resorcinol         |    |
| $R=naphthetyl, R_1=alkyl$                  | 65 |
| $n,y,z=1$                                  |    |
| Octylthiomethyl naphthetyl naphthol        |    |
| $n,y=1, z=2$                               |    |
| Di (octylthiomethyl) naphthetyl naphthol   | 70 |
| $n=3, y,z=1$                               |    |
| Octylthiomethyl naphthetyl pyrogallol      |    |
| $n=2, y=1, z=2$                            | 75 |
| Di (octylthiomethyl) naphthetyl resorcinol |    |

## 4

|                                                |    |
|------------------------------------------------|----|
| $R=alkyl, R_1=aryl$                            |    |
| $n,y,z=1$                                      |    |
| Phenylthiomethyl octyl phenol                  |    |
| $n,y=1, z=2$                                   |    |
| Di (phenylthiomethyl) octyl phenol             |    |
| $n=1, y,z=2$                                   |    |
| Di (phenylthiomethyl) dioctyl phenol           |    |
| $n=2, y,z=1$                                   |    |
| Phenolthiomethyl undecyl resorcinol            |    |
| $n=2, y=1, z=2$                                |    |
| Di (phenylthiomethyl) undecyl resorcinol       |    |
| $n,y=2, z=1$                                   |    |
| Phenylthiomethyl dioctyl resorcinol            |    |
| $R=hydrogen, R_1=aryl$                         |    |
| $n=1, y=3, z=2$                                | 20 |
| Di (phenylthiomethyl) phenol                   |    |
| $n=1, y=2, z=3$                                |    |
| Tri (phenylthiomethyl) phenol                  |    |
| $n,y,z=2$                                      | 25 |
| Di (phenylthiomethyl) resorcinol               |    |
| $R=alkyl, R_1=cyclohexyl$                      |    |
| $n,y,z=1$                                      | 30 |
| Cyclohexylthiomethyl octadecyl naphthol        |    |
| $n,y=1, z=2$                                   |    |
| Di (cyclohexylthiomethyl) octadecyl naphthol   |    |
| $n=1, y,z=2$                                   | 35 |
| Di (cyclohexylthiomethyl) dioctadecyl naphthol |    |
| $n=1, y=2, z=1$                                |    |
| Cyclohexylthiomethyl diamyl phenol             |    |
| $n=2, y,z=1$                                   | 40 |
| Cyclohexylthiomethyl octyl resorcinol          |    |
| $n=2, y=1, z=2$                                |    |
| Di (cyclohexylthiomethyl) octyl resorcinol     |    |
| $n,y=2, z=1$                                   | 45 |
| Cyclohexylthiomethyl dioctyl resorcinol        |    |
| $R=hydrogen, R_1=cycloalkyl$                   |    |
| $n=1, y=3, z=2$                                | 50 |
| Di (cyclohexylthiomethyl) phenol               |    |
| $n=1, y=2, z=3$                                |    |
| Tri (cyclohexylthiomethyl) phenol              |    |
| $n=3, y=1, z=2$                                | 55 |
| Di (cyclohexylthiomethyl) pyrogallol           |    |
| $n,y,z=2$                                      |    |
| Di (cyclohexylthiomethyl) hydroquinone         |    |
| $R=alkyl, R_1=aralkyl$                         | 60 |
| $n,y,z=1$                                      |    |
| Benzylthiomethyl octyl phenol                  |    |
| $n,y=1, z=2$                                   |    |
| Di (benzylthiomethyl) octyl phenol             |    |
| $n=1, y=2, z=1$                                |    |
| Benzylthiomethyl dioctyl phenol                |    |
| $n=1, y,z=2$                                   |    |
| Di (benzylthiomethyl) dioctyl phenol           |    |
| $n=2, y,z=1$                                   | 75 |
| Benzylthiomethyl undecyl hydroquinone          |    |

$n=2, y=1, z=2$ 

Di (benzylthiomethyl) undecyl hydroquinone

 $n,y=2, z=1$ 

Benzylthiomethyl diundecyl hydroquinone

 $R=hydrogen, R_1=aralkyl$  $n=1, y=3, z=2$ 

Di (benzylthiomethyl) phenol

 $n=1, y=2, z=3$ 

Tri (benzylthiomethyl) phenol

 $n,y,z=2$ 

Di (benzylthiomethyl) resorcinol

 $R=alkyl, R_1=naphthetyl$  $n,y,z=1$ 

Naphthenthylthiomethyl octyl naphthol

 $n,y=1, z=2$ 

Di (naphthenthylthiomethyl) octyl naphthol

 $n=1, y=2, z=1$ 

Naphthenthylthiomethyl dioctyl naphthol

 $n=2, y,z=1$ 

Naphthenthylthiomethyl undecyl resorcinol

 $n=2, y=1, z=2$ 

Di (naphthenthylthiomethyl) undecyl resorcinol

 $R=hydrogen, R_1=naphthetyl$  $n=1, y=3, z=2$ 

Di (naphthenthylthiomethyl) phenol

 $n=1, y=2, z=3$ 

Tri (naphthenthylthiomethyl) phenol

 $n,y,z=2$ 

Di (naphthenthylthiomethyl) resorcinol

 $R=tertiary aminomethyl, R_1=alkyl$  $n=1, y=2, z=1$ 

Amylthiomethyl di (dimethylaminomethyl) phenol

 $n=1, y=1, z=2$ 

Di (amylthiomethyl) dimethylaminomethyl phenol

 $n=2, y=1, z=1$ 

Amylthiomethyl morpholinomethyl resorcinol

Any of the known classical methods of synthesis may be used in the preparation of these compounds and the following reactions are given as illustrating two of the methods preferable to the present invention. The first is the reaction of a mercaptan and a dimethyl amino methyl derivative of a hydroxy aromatic compound:



The second is the reaction of an alkylated phenol, formaldehyde, and a mercaptan, as follows:



## Example I

In preparing amylthiomethyl octyl phenol according to reaction No. 1, 106 grams of dimethylaminomethyl octyl phenol and 210 grams of amyl mercaptan were intimately mixed with agitation and refluxed for 35 hours. Dimethylamine was given off and after the evolution was complete, the reaction mixture was transferred to a distilling flask and distilled under vacuum. The product was collected at 150 to 190° C. at three millimeters pressure. The resulting amylthiomethyl octyl phenol was obtained as a clear, light yellow liquid (B. P. 160-170° C. at three millimeters mercury) and analyzed 9.3% sulfur.

## Example II

65 grams of amylthiomethyl octyl phenol, 22 grams of barium hydroxide, and 250 cc. of toluene were intimately mixed under agitation and refluxed under an automatic water separator until no more water was eliminated from the reaction. Filter-cel was added to the reaction mixture and the excess barium hydroxide filtered out. The filtrate was freed of toluene by heating under vacuum and the resulting barium amylthiomethyl octyl phenolate was obtained as a clear, brittle, light-brown solid, which was dissolved in an equal weight of lubricating oil. The 50% concentrate analyzed 8.3% barium and 4.35% sulfur.

## Example III

13 grams of magnesium ribbon was stirred with 200 cc. absolute ethyl alcohol and 200 cc. absolute methyl alcohol until the metal was substantially dissolved. 160 grams of amylthiomethyl octyl phenol was added and the alcohol solvent substantially distilled off. Toluene was added and then distilled off to eliminate the remaining portions of alcohol solvent. Additional toluene was added and the solution was filtered through clay. The solvent was removed by distillation under vacuum and the residue dissolved in an equal weight of hydrocarbon oil. The resulting concentrate of magnesium amylthiomethyl octyl phenol in an equal weight of hydrocarbon oil analyzed 5.2% ash.

## Example IV

A partially substituted product was obtained by reacting tri (dimethylaminomethyl) phenol under mild conditions in accordance with reaction No. 1. In this reaction, 265 grams of tri (dimethylaminomethyl) phenol, 500 grams of amyl mercaptan, and 400 cc. of toluene were stirred together and refluxed for 60 hours. Dimethylamine was given off and after the evolution was complete, the toluene and excess amyl mercaptan were distilled off at atmospheric pressure and a small intermediate fraction was collected which boiled up to 150° C. at 10 millimeters mercury. The residual amylthiomethyl di (dimethylaminomethyl) phenol appeared as a light brown oil and analyzed 7.42% sulfur and 9.02% nitrogen.

## Example V

In preparing tri (benzylthiomethyl) phenol according to reaction No. 1, 133 grams of tri (dimethylaminomethyl) phenol and 186 grams benzyl mercaptan were intimately mixed with agitation and heated to 140-145° C. for three hours. Upon completion of the evolution of dimethyl amine, the product was filtered through clay and the resulting tri (benzylthiomethyl) phenol was obtained as a clear greenish-yellow oily liquid which analyzed 16.2% sulfur.

7  
Example VI

In preparing the barium salt of tri (benzylthiomethyl) phenol of Example V, 50 grams of the product of Example V, 17 grams barium hydroxide, and 300 cc. toluene were stirred together and refluxed under an automatic water separator. The product was filtered through clay and the solvent removed by heating in vacuum. A resulting barium tri (benzylthiomethyl) phenolate was obtained as a clear light brown viscous residue which analyzed 17.7% ash.

Obviously many modifications and variations of the invention as herein set forth may be made without departing from the spirit and the scope thereof, and, therefore, only such limitations should be imposed as are indicated in the appended claims.

We claim:

1. As a new compound, di (dimethylamino-methyl) amylthiomethyl phenol.
2. Barium (amylthiomethyl) octyl phenolate.
3. As a composition of matter a compound possessing the structure.



in which Y and Z are alkyl groups and X is a member of the class consisting of hydrogen and metal equivalents thereof.

4. As a composition of matter a compound possessing the structure



in which X is a member of the class consisting of hydrogen and metal equivalents thereof, Y and Z are alkyl groups; and m and n are small integers.

5. An aromatic methylene thioether having the following general formula



wherein R is a radical selected from the group consisting of hydrogen and a hydrocarbon radical, R<sub>1</sub> is a hydrocarbon radical, X is a substituent selected from the group consisting of hydroxyl radicals and metal substituted hydroxyl radicals and n, y, and z are integers of at least one.

6. An aromatic methylene thioether having the following general formula



10 wherein R is a radical selected from the group consisting of hydrogen and a hydrocarbon radical, R<sub>1</sub> is a hydrocarbon radical and y and z are integers of at least one.

7. An aromatic methylene thioether having the following general formula



20 wherein R is a radical selected from the group consisting of hydrogen and a hydrocarbon radical, R<sub>1</sub> is a hydrocarbon radical, M is a metal equivalent and y and z are integers of at least 25 one.

8. A method of preparing an aromatic methylene thioether which comprises reacting an aromatic compound containing at least one hydroxyl radical with formaldehyde and an alkyl mercaptan.

9. A method of preparing an aromatic methylene thioether which comprises reacting an aromatic compound containing a hydroxyl radical with formaldehyde and an alkyl mercaptan and thereafter converting the free hydroxyl radical to its corresponding metal salt.

10. A method of preparing an aromatic methylene thioether which comprises reacting an alkyl phenol with formaldehyde and an alkyl mercaptan.

RUSH F. McCLEARY.  
STILES M. ROBERTS.

## REFERENCES CITED

45 The following references are of record in the file of this patent:

## UNITED STATES PATENTS

|    | Number    | Name          | Date          |
|----|-----------|---------------|---------------|
| 50 | 2,111,260 | Brunner       | Mar. 15, 1938 |
|    | 2,223,693 | Martin et al. | Dec. 3, 1940  |
|    | 2,249,626 | Cook et al.   | July 15, 1941 |

## FOREIGN PATENTS

|    | Number  | Country            | Date          |
|----|---------|--------------------|---------------|
| 55 | 450,760 | British to Johnson | July 20, 1936 |

## OTHER REFERENCES

Manchot, "Annalen," vol. 345, pages 322-323.  
Baumann, "Berichte," vol. 24, page 1446.